



US007030192B2

(12) **United States Patent**  
**Rajagopalan et al.**

(10) **Patent No.:** **US 7,030,192 B2**  
(45) **Date of Patent:** **Apr. 18, 2006**

- (54) **GOLF BALL CORES COMPRISING A HALOGENATED ORGANOSULFUR COMPOUND**
- (75) Inventors: **Murali Rajagopalan**, South Dartmouth, MA (US); **David A. Bulpett**, Boston, MA (US); **Douglas S. Goguen**, New Bedford, MA (US); **Derek A. Ladd**, Acushnet, MA (US)
- (73) Assignee: **Acushnet Company**, Fairhaven, MA (US)
- (\*) Notice: Subject to any disclaimer, the term of this patent is extended or adjusted under 35 U.S.C. 154(b) by 115 days.
- (21) Appl. No.: **10/867,079**
- (22) Filed: **Jun. 14, 2004**
- (65) **Prior Publication Data**  
US 2004/0225068 A1 Nov. 11, 2004

**Related U.S. Application Data**

- (63) Continuation-in-part of application No. 10/437,694, filed on May 14, 2003, which is a continuation-in-part of application No. 09/951,963, filed on Sep. 13, 2001, now Pat. No. 6,635,716.
- (51) **Int. Cl.**  
*A63B 37/06* (2006.01)
- (52) **U.S. Cl.** ..... **525/261**; 525/274; 473/372; 473/373; 473/377
- (58) **Field of Classification Search** ..... None  
See application file for complete search history.

(56) **References Cited**

U.S. PATENT DOCUMENTS

- 5,252,652 A 10/1993 Egashira et al. ..... 524/392  
5,605,968 A 2/1997 Egashira et al. ..... 525/221  
5,697,856 A 12/1997 Moriyama et al. ..... 473/374  
5,711,723 A 1/1998 Hiraoka et al. ..... 473/374  
5,776,012 A 7/1998 Moriyama et al. ..... 473/372  
5,779,563 A 7/1998 Yamagishi et al. ..... 473/371  
5,816,944 A 10/1998 Asakura et al. ..... 473/372  
5,872,185 A 2/1999 Ichikawa et al. ..... 525/93  
5,877,264 A 3/1999 Logothetis et al. ..... 526/86  
5,919,101 A 7/1999 Yokota et al. ..... 473/372  
5,929,171 A 7/1999 Sano et al. ..... 525/261  
5,977,264 A 11/1999 Ichikawa et al. ..... 525/329.9

- 5,994,472 A 11/1999 Egashira et al. ..... 525/221  
6,120,392 A 9/2000 Kashiwagi et al. ..... 473/374  
6,121,357 A 9/2000 Yokota ..... 524/406  
6,126,558 A 10/2000 Higuchi et al. ..... 473/374  
6,129,640 A 10/2000 Higuchi et al. ..... 473/374  
6,135,898 A 10/2000 Higuchi et al. ..... 473/374  
6,174,247 B1 1/2001 Higuchi et al. ..... 473/374  
6,184,301 B1 2/2001 Shindo et al. ..... 525/261  
6,210,292 B1 4/2001 Higuchi et al. ..... 473/374  
6,213,896 B1 4/2001 Higuchi et al. ..... 473/374  
6,231,460 B1 5/2001 Higuchi et al. ..... 473/374  
6,241,625 B1 6/2001 Yokota et al. ..... 473/373  
6,244,978 B1 6/2001 Higuchi et al. ..... 473/374  
6,248,028 B1 6/2001 Higuchi et al. ..... 473/374  
6,267,692 B1 7/2001 Higuchi et al. ..... 473/365  
6,267,694 B1 \* 7/2001 Higuchi et al. ..... 473/374  
6,287,218 B1 9/2001 Obama ..... 473/377  
6,299,551 B1 10/2001 Higuchi et al. ..... 473/374  
6,849,006 B1 \* 2/2005 Cavallaro et al. ..... 473/376  
6,960,630 B1 \* 11/2005 Cavallaro et al. ..... 525/261  
2001/0011045 A1 8/2001 Takemura et al. ..... 473/371  
2001/0016522 A1 8/2001 Watanabe et al. ..... 473/371  
2001/0018374 A1 8/2001 Ichikawa et al. ..... 473/367  
2001/0031669 A1 10/2001 Obama ..... 473/371  
2001/0031673 A1 10/2001 Watanabe ..... 473/378  
2005/0250601 A1 \* 11/2005 Kim et al. ..... 473/371

FOREIGN PATENT DOCUMENTS

GB 1222738 \* 2/1971

\* cited by examiner

*Primary Examiner*—David J. Buttner

(74) *Attorney, Agent, or Firm*—William B. Lacy

(57) **ABSTRACT**

A golf ball comprising a core having a diameter of between about 1.54 inches and about 1.57 inches, a compression of between about 70 and 80, and comprising a polybutadiene rubber composition comprising a magnesium salt of pentachlorothiophenol; a cover having a thickness of about 0.04 inches or less and comprising a castable polyurethane or polyurea composition; and an inner cover layer disposed between the core and the outer cover layer, the inner cover layer having a thickness of about 0.04 inches or less and selected from the group consisting of ionomers, vinyl resins, polyolefins, polyurethanes, polyureas, polyamides, acrylic resins, thermoplastics, polyphenylene oxide resins, thermoplastic polyesters, thermoplastic rubbers, partially-neutralized polymers, highly-neutralized polymers, and fully-neutralized polymers.

**21 Claims, No Drawings**

## 1

**GOLF BALL CORES COMPRISING A HALOGENATED ORGANOSULFUR COMPOUND**

**CROSS REFERENCE TO RELATED APPLICATIONS**

This application is a continuation-in-part of co-pending U.S. application Ser. No. 10/437,694, filed May 14, 2003, which is a continuation-in-part of Ser. No. 09/951,963 U.S. Pat. No. 6,635,716, filed Sep. 13, 2001.

**FIELD OF THE INVENTION**

This invention relates generally to golf balls and, in particular, golf ball cores formed of a polymer composition including a halogenated organosulfur compound.

**BACKGROUND**

Conventional golf balls can be divided into two general classes: solid and wound. Solid golf balls include one-piece, two-piece (i.e., solid core and a cover), and multi-layer (i.e., solid core of one or more layers and/or a cover of one or more layers) golf balls. Wound golf balls typically include a solid, hollow, or fluid-filled center, surrounded by a tensioned elastomeric material, and a cover. Solid balls have traditionally been considered longer and more durable than wound balls, but also lack a particular "feel" provided by the wound construction.

By altering ball construction and composition, manufacturers can vary a wide range of playing characteristics, such as compression, velocity, and spin, each of which can be optimized for various playing abilities. One golf ball component, in particular, that many manufacturers are continually looking to improve is the center or core. The core becomes the "engine" of the golf ball when hit with a club head. Generally, golf ball cores and/or centers are constructed with a polybutadiene-based polymer composition. Compositions of this type are constantly being altered in an effort to provide a higher coefficient of restitution ("COR") while at the same time resulting in a lower compression which, in turn, can lower the golf ball spin rate, provide better "feel," or both. This is a difficult task, however, given the physical limitations of currently-available polymers. As such, there remains a need for novel and improved golf ball core compositions.

It has been determined that, upon that addition of a halogenated organosulfur compound or the salts thereof, in particular, pentachlorothiophenol ("PCTP") salt, to polybutadiene rubber compositions, that golf ball cores may be constructed that exhibit increased COR, decreased compression, or both. The present invention is, therefore, directed to golf ball centers and cores that include a halogenated organosulfur compound, or a salt thereof, for embodiments such as these.

**SUMMARY OF THE INVENTION**

The present invention is directed to a golf ball formed of a core and a cover, wherein the core has a diameter of at least about 1.50 inches and comprises a polybutadiene rubber composition comprising at least about 2.2 parts per hundred of a halogenated organosulfur compound, and wherein the cover has a thickness of less than about 0.1 inches and comprises a polyurethane composition.

## 2

The core can include a center and an outer core layer and the core preferably has a diameter of at least about 1.55 inches. The cover may include an inner cover layer and an outer cover layer and, preferably, at least one of the inner and outer cover layers has a thickness of less than about 0.05 inches. The inner cover layer may include an ionomeric material, vinyl resins, polyolefins, polyurethanes, polyureas, polyamides, acrylic resins, thermoplastics, polyphenylene oxide resins, thermoplastic polyesters, thermoplastic rubbers, fully-neutralized polymers, partially-neutralized polymers, and mixtures thereof.

The polybutadiene rubber composition may include between about 2.2 parts and about 5 parts of a halogenated organosulfur compound. The halogenated organosulfur compound may include pentafluorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol 2,3,4-fluorothiophenol; 3,4,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; pentabromothiophenol; 2-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,4,5-tetraiodothiophenol; 2,3,5,6-tetraiodothiophenol; and their zinc salts, the metal salts thereof, and mixtures thereof, but is preferably pentachlorothiophenol or the metal salt thereof. The metal salt may be zinc, calcium, potassium, magnesium, sodium, and lithium, but is preferably zinc.

In one embodiment, the core has a compression less than about 75 and the golf ball has a coefficient of restitution of greater than about 0.800. In another, the core has a compression less than about 75 and the golf ball has a coefficient of restitution of greater than about 0.815. In still another, the core has a compression less than about 55 and the golf ball has a coefficient of restitution of greater than about 0.800.

The polybutadiene composition may further include an  $\alpha,\beta$ -unsaturated carboxylic acid or a metal salt thereof, an organic peroxide, and a filler. If the outer cover layer includes polyurethane, it includes a prepolymer formed of a polyisocyanate and a polyol, and a curing agent. Preferably, at least one of the prepolymer and curing agent are saturated. In an alternative embodiment, the polyurethane composition comprises at least one of a UV absorber, a hindered amine light stabilizer, or an optical brightener.

The present invention is also directed to a golf ball formed of a core and a cover, wherein the core has a diameter of at least about 1.50 inches and comprises a polybutadiene rubber composition comprising at least about 2.2 parts per hundred of a halogenated organosulfur compound, and wherein the cover has a thickness of less than about 0.1 inches and is formed of an inner cover layer and an outer cover layer.

In one embodiment, the core comprises a center having an outer diameter of at least about 1.55 inches and an outer core layer. It is preferred that at least one of the inner and outer cover layers have a thickness of less than about 0.05 inches. Either of the cover layers may include vinyl resins, polyolefins, polyurethanes, polyureas, polyamides, acrylic resins, thermoplastics, polyphenylene oxide resins, thermoplastic polyesters, thermoplastic rubbers, fully-neutralized polymers, partially-neutralized polymers, and mixtures thereof.

The polybutadiene rubber composition preferably includes between about 2.2 parts and about 5 parts of a halogenated organosulfur compound. The halogenated organosulfur compound can be pentafluorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol 2,3,4-fluorothiophenol; 3,4,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; pentabromothiophenol; 2-bromo-2,3-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,4,5-tetraiodothiophenol; 2,3,5,6-tetraiodothiophenol; and their zinc salts, the metal salts thereof, and mixtures thereof, and preferably is pentachlorothiophenol or the metal salt thereof. The metal salt is selected from the group consisting of zinc, calcium, potassium, magnesium, sodium, and lithium and is preferably zinc.

The core compression is preferably less than about 75 and the golf ball coefficient of restitution preferably greater than about 0.800. In one embodiment, the core has a compression less than about 75 and the golf ball has a coefficient of restitution of greater than about 0.815. In another, the core has a compression less than about 55 and the golf ball has a coefficient of restitution of greater than about 0.800. In still another, the polybutadiene composition further comprises an  $\alpha,\beta$ -unsaturated carboxylic acid or a metal salt thereof, an organic peroxide, and a filler.

In another embodiment, the outer cover layer is formed of a polyurethane composition comprising a prepolymer formed of a polyisocyanate and a polyol, and a curing agent. At least one of the prepolymer and curing agent are saturated. In a preferred embodiment, the polyurethane composition comprises at least one of a UV absorber, a hindered amine light stabilizer, or an optical brightener.

The present invention is also directed to a golf ball formed of a core and a cover, wherein the core has a diameter of at least about 1.55 inches and comprises a polybutadiene rubber composition comprising greater than about 2.3 parts per hundred of pentachlorothiophenol or a metal salt thereof, and wherein the cover comprises an inner cover layer comprising an ionomeric material and having a thickness of less than about 0.04 inches; and an outer cover layer having a thickness of less than about 0.04 inches and comprising a polyurethane composition.

## DETAILED DESCRIPTION

The golf ball cores of the present invention may comprise any of a variety of constructions but preferably includes a core and a cover surrounding the core. The core and/or the cover may have more than one layer and an intermediate layer may be disposed between the core and the cover of the golf ball. For example, the core of the golf ball may comprise a conventional center surrounded by an intermediate or outer core layer disposed between the center and the inner cover layer. The core may be a single layer or may comprise a plurality of layers. The innermost portion of the core may be solid or it may be a liquid filled sphere, but preferably it is solid. As with the core, the intermediate layer or outer core layer may also comprise a plurality of layers. The core may also comprise a solid or liquid filled center around which many yards of a tensioned elastomeric material are wound.

The materials for solid cores include compositions having 20 a base rubber, a crosslinking agent, a filler, a halogenated organosulfur compound, and a co-crosslinking or initiator agent. The base rubber typically includes natural or synthetic rubbers. A preferred base rubber is 1,4-polybutadiene having a cis-structure of at least 40%, more preferably at least about 90%, and most preferably at least about 95%. Most preferably, the base rubber comprises high-Mooney-viscosity rubber. Preferably, the base rubber has a Mooney viscosity greater than about 35, more preferably greater than about 40, most preferably greater than about 50. Preferably, the polybutadiene rubber has a molecular weight greater than about 400,000 and a polydispersity of no greater than about 2. Examples of desirable polybutadiene rubbers include BUNA® CB22 and BUNA® CB23, commercially available from Bayer of Akron, Ohio; UBEPOL® 360L and UBE-35 POL® 150L, commercially available from UBE Industries of Tokyo, Japan; and CARIFLEX® BCP820 and CARIFLEX® BCP824, commercially available from Shell of Houston, Tex. If desired, the polybutadiene can also be mixed with other elastomers known in the art such as natural 40 rubber, polyisoprene rubber and/or styrene-butadiene rubber in order to modify the properties of the core.

The crosslinking agent includes a metal salt, such as a zinc salt or a magnesium unsaturated fatty acid, such as acrylic or methacrylic acid, having 3 to 8 carbon atoms. Examples include, but are not limited to, one or more metal salt diacrylates, dimethacrylates, and monomethacrylates, wherein the metal is magnesium, calcium, zinc, aluminum, sodium, lithium, or nickel. Preferred acrylates include zinc acrylate, zinc diacrylate, zinc methacrylate, zinc 50 dimethacrylate, and mixtures thereof. The crosslinking agent is typically present in an amount greater than about 10 parts per hundred ("pph") parts of the base polymer, preferably from about 20 to 40 pph of the base polymer, more preferably from about 25 to 35 pph of the base polymer.

The initiator agent can be any known polymerization initiator which decomposes during the cure cycle. Suitable initiators include organic peroxide compounds, such as dicumyl peroxide; 1,1-di(t-butylperoxy) 3,3,5-trimethyl cyclohexane;  $\alpha,\alpha$ -bis (t-butylperoxy) diisopropylbenzene; 2,5-dimethyl-2,5-di(t-butylperoxy) hexane; di-t-butyl peroxide; and mixtures thereof. Other examples include, but are not limited to, VAROX® 231XL and Varox® DCP-R, commercially available from Elf Atochem of Philadelphia, Pa.; PERKODOX® BC and PERKODOX® 14, commercially available from Akzo Nobel of Chicago, Ill.; and ELASTOCHEM® DCP-70, commercially available from Rhein Chemie of Trenton, N.J.

It is well known that peroxides are available in a variety of forms having different activity. The activity is typically defined by the "active oxygen content." For example, PERKODOX® BC peroxide is 98% active and has an active oxygen content of 5.80%, whereas PERKODOX® DCP-70 is 70% active and has an active oxygen content of 4.18%. If the peroxide is present in pure form, it is preferably present in an amount of at least about 0.25 pph, more preferably between about 0.35 pph and about 2.5 pph, and most preferably between about 0.5 pph and about 2 pph. Peroxides are also available in concentrate form, which are well-known to have differing activities, as described above. In this case, if concentrate peroxides are employed in the present invention, one skilled in the art would know that the concentrations suitable for pure peroxides are easily adjusted for concentrate peroxides by dividing by the activity. For example, 2 pph of a pure peroxide is equivalent 4 pph of a concentrate peroxide that is 50% active (i.e., 2 divided by 0.5=4).

The halogenated organosulfur compounds of the present invention include, but are not limited to those having the following general formula:



where at least one of R<sub>1</sub>-R<sub>5</sub> is a halogen and where R<sub>1</sub>-R<sub>5</sub> can alternatively be C<sub>1</sub>-C<sub>8</sub> alkyl groups; halogen groups; thiol groups (—SH), carboxylated groups; sulfonated groups; and hydrogen; in any order; and also pentafluorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol; 2,3,4-fluorothiophenol; 3,4,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; pentabromothiophenol; 2-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,4,5-tetraiodothiophenol; 2,3,5,6-tetraiodothiophenol and; and their zinc salts. Preferably, the halogenated organosulfur compound is pentachlorothiophenol, which is commercially available in neat form or under the tradename STRUKTOL®, a clay-based carrier containing the sulfur compound pentachlorothiophenol loaded at 45 percent (correlating to 2.4 parts PCTP). STRUKTOL® is commercially available from Struktol Company of America of Stow, Ohio. PCTP is commercially available in neat form from eChinachem of

San Francisco, Calif. and in the salt form from eChinachem of San Francisco, Calif. Most preferably, the halogenated organosulfur compound is the zinc salt of pentachlorothiophenol, which is commercially available from eChinachem of San Francisco, Calif. The halogenated organosulfur compounds of the present invention are preferably present in an amount greater than about 2.2 pph, more preferably between about 2.3 pph and about 5 pph, and most preferably between about 2.3 and about 4 pph.

- 10 Fillers typically include materials such as tungsten, zinc oxide, barium sulfate, silica, calcium carbonate, zinc carbonate, metals, metal oxides and salts, regrind (recycled core material typically ground to about 30 mesh particle), high-Mooney-viscosity rubber regrind, and the like. Fillers added to one or more portions of the golf ball typically include processing aids or compounds to affect rheological and mixing properties, density-modifying fillers, tear strength, or reinforcement fillers, and the like. The fillers are generally inorganic, and suitable fillers include numerous metals or 15 metal oxides, such as zinc oxide and tin oxide, as well as barium sulfate, zinc sulfate, calcium carbonate, barium carbonate, clay, tungsten, tungsten carbide, an array of silicas, and mixtures thereof. Fillers may also include various foaming agents or blowing agents which may be readily selected by one of ordinary skill in the art. Fillers may include polymeric, ceramic, metal, and glass microspheres 20 may be solid or hollow, and filled or unfilled. Fillers are typically also added to one or more portions of the golf ball to modify the density thereof to conform to uniform golf ball 25 standards. Fillers may also be used to modify the weight of the center or at least one additional layer for specialty balls, e.g., a lower weight ball is preferred for a player having a low swing speed.

The invention also includes a method to convert the 30 cis-isomer of the polybutadiene resilient polymer component to the trans-isomer during a molding cycle and to form a golf ball. A variety of methods and materials suitable for cis-to-trans conversion have been disclosed in U.S. Pat. No. 6,162,135 and U.S. application Ser. Nos. 09/461,736, filed Dec. 16, 1999; 09/458,676, filed Dec. 10, 1999; and 09/461, 40 421, filed Dec. 16, 1999, each of which are incorporated herein, in their entirety, by reference.

The materials used in forming either the golf ball center or any portion of the core, in accordance with the invention, 45 may be combined to form a mixture by any type of mixing known to one of ordinary skill in the art. Suitable types of mixing include single pass and multi-pass mixing. Suitable mixing equipment is well known to those of ordinary skill in the art, and such equipment may include a Banbury mixer, a two-roll mill, or a twin screw extruder.

Conventional mixing speeds for combining polymers are 50 typically used. The mixing temperature depends upon the type of polymer components, and more importantly, on the type of free-radical initiator. Suitable mixing speeds and temperatures are well-known to those of ordinary skill in the art, or may be readily determined without undue experimentation.

The mixture can be subjected to, e.g., a compression or 55 injection molding process, to obtain solid spheres for the center or hemispherical shells for forming an intermediate layer. The temperature and duration of the molding cycle are selected based upon reactivity of the mixture. The molding cycle may have a single step of molding the mixture at a single temperature for a fixed time duration. The molding cycle may also include a two-step process, in which the polymer mixture is held in the mold at an initial temperature for an initial duration of time, followed by holding at a

second, typically higher temperature for a second duration of time. In a preferred embodiment of the current invention, a single-step cure cycle is employed. The materials used in forming either the golf ball center or any portion of the core, in accordance with the invention, may be combined to form a golf ball by an injection molding process, which is also well-known to one of ordinary skill in the art. Although the curing time depends on the various materials selected, those of ordinary skill in the art will be readily able to adjust the curing time upward or downward based on the particular materials used and the discussion herein.

Properties that are desirable for the cover include good moldability, high abrasion resistance, high tear strength, high resilience, and good mold release. The cover typically has a thickness to provide sufficient strength, good performance characteristics, and durability. The cover preferably has a thickness of less than about 0.1 inches, more preferably, less than about 0.05 inches, and most preferably, between about 0.02 inches and about 0.04 inches. The invention is particularly directed towards a multilayer golf ball which comprises a core, an inner cover layer, and an outer cover layer. In this embodiment, preferably, at least one of the inner and outer cover layer has a thickness of less than about 0.05 inches, more preferably between about 0.02 inches and about 0.04 inches. Most preferably, the thickness of either layer is about 0.03 inches.

When the golf ball of the present invention includes an inner cover layer, this layer can include any materials known to those of ordinary skill in the art, including thermoplastic and thermosetting material, but preferably the inner cover can include any suitable materials, such as ionic copolymers of ethylene and an unsaturated monocarboxylic acid which are available under the trademark SURLYN of E.I. DuPont de Nemours & Co., of Wilmington, Del., or IOTEK or ESCOR of Exxon. These are copolymers or terpolymers of ethylene and methacrylic acid or acrylic acid partially neutralized with salts of zinc, sodium, lithium, magnesium, potassium, calcium, manganese, nickel or the like, in which the salts are the reaction product of an olefin having from 2 to 8 carbon atoms and an unsaturated monocarboxylic acid having 3 to 8 carbon atoms. The carboxylic acid groups of the copolymer may be totally or partially neutralized and might include methacrylic, crotonic, maleic, fumaric or itaconic acid.

This golf ball can likewise include one or more homopolymeric or copolymeric inner cover materials, such as:

(1) Vinyl resins, such as those formed by the polymerization of vinyl chloride, or by the copolymerization of vinyl chloride with vinyl acetate, acrylic esters or vinylidene chloride;

(2) Polyolefins, such as polyethylene, polypropylene, polybutylene and copolymers such as ethylene methylacrylate, ethylene ethylacrylate, ethylene vinyl acetate, ethylene methacrylic or ethylene acrylic acid or propylene acrylic acid and copolymers and homopolymers produced using a single-site catalyst or a metallocene catalyst;

(3) Polyurethanes, such as those prepared from polyols and diisocyanates or polyisocyanates and those disclosed in U.S. Pat. No. 5,334,673;

(4) Polyureas, such as those disclosed in U.S. Pat. No. 5,484,870;

(5) Polyamides, such as poly(hexamethylene adipamide) and others prepared from diamines and dibasic acids, as well as those from amino acids such as poly(caprolactam), and

blends of polyamides with SURLYN, polyethylene, ethylene copolymers, ethyl-propylene-non-conjugated diene terpolymer, and the like;

(6) Acrylic resins and blends of these resins with polyvinyl chloride, elastomers, and the like;

(7) Thermoplastics, such as urethanes; olefinic thermoplastic rubbers, such as blends of polyolefins with ethylene-propylene-non-conjugated diene terpolymer; block copolymers of styrene and butadiene, isoprene or ethylene-butylene rubber; or copoly(ether-amide), such as PEBAK, sold by ELF Atochem of Philadelphia, Pa.;

(8) Polyphenylene oxide resins or blends of polyphenylene oxide with high impact polystyrene as sold under the trademark NORYL by General Electric Company of Pittsfield, Mass.;

(9) Thermoplastic polyesters, such as polyethylene terephthalate, polybutylene terephthalate, polyethylene terephthalate/glycol modified and elastomers sold under the trademarks HYTREL by E.I. DuPont de Nemours & Co. of Wilmington, Del., and LOMOD by General Electric Company of Pittsfield, Mass.;

(10) Blends and alloys, including polycarbonate with acrylonitrile butadiene styrene, polybutylene terephthalate, polyethylene terephthalate, styrene maleic anhydride, polyethylene, elastomers, and the like, and polyvinyl chloride with acrylonitrile butadiene styrene or ethylene vinyl acetate or other elastomers; and

(11) Blends of thermoplastic rubbers with polyethylene, propylene, polyacetal, nylon, polyesters, cellulose esters, and the like.

Preferably, the inner cover includes polymers, such as ethylene, propylene, butene-1 or hexane-1 based homopolymers or copolymers including functional monomers, such as acrylic and methacrylic acid and fully or partially neutralized ionomer resins and their blends, methyl acrylate, methyl methacrylate homopolymers and copolymers, imidized, amino group containing polymers, polycarbonate, reinforced polyamides, polyphenylene oxide, high impact polystyrene, polyether ketone, polysulfone, poly(phenylene sulfide), acrylonitrile-butadiene, acrylic-styrene-acrylonitrile, poly(ethylene terephthalate), poly(butylene terephthalate), poly(ethylene vinyl alcohol), poly(tetrafluoroethylene) and their copolymers including functional comonomers, and blends thereof. Suitable cover compositions also include a polyether or polyester thermoplastic urethane, a thermoset polyurethane, a low modulus ionomer, such as acid-containing ethylene copolymer ionomers, including E/X/Y terpolymers where E is ethylene, X is an acrylate or methacrylate-based softening comonomer present in about 0 to 50 weight percent and Y is acrylic or methacrylic acid present in about 5 to 35 weight percent. Preferably, the acrylic or methacrylic acid is present in about 8 to 35 weight percent, more preferably 8 to 25 weight percent, and most preferably 8 to 20 weight percent.

To prevent or minimize the penetration of moisture, typically water vapor, into core of golf ball, an intermediate moisture vapor barrier layer may also be disposed around core. Preferably, the moisture vapor barrier layer preferably has a moisture vapor transmission rate that is lower than that of the cover, and more preferably less than the moisture vapor transmission rate of an ionomer resin such as Surlyn®, which is in the range of about 0.45 to about 0.95 (g·mm)/(m<sup>2</sup>·day). The moisture vapor transmission rate is defined as the mass of moisture vapor that diffuses into a material of a given thickness per unit area per unit time. The preferred standards of measuring the moisture vapor transmission rate include ASTM F1249-90 entitled "Standard

Test Method for Water Vapor Transmission Rate Through Plastic Film and Sheeting Using a Modulated Infrared Sensor," and ASTM F372-99 entitled "Standard Test Method for Water Vapor Transmission Rate of Flexible Barrier Materials Using an Infrared Detection Technique," among others. In accordance to one aspect of the invention, the moisture vapor barrier layer can be of any material disclosed herein meeting the desired vapor transmission rate.

Any of the inner or outer cover layers may also be formed from polymers containing  $\alpha,\beta$ -unsaturated carboxylic acid groups, or the salts thereof, that have been 100 percent neutralized by salts of organic fatty acids and a suitable cation source. The acid moieties of the highly-neutralized polymers ("HNP"), typically ethylene-based ionomers, are preferably neutralized greater than about 70%, more preferably greater than about 90%, and most preferably at least about 100%. The HNP's can be also be blended with a second polymer component, which, if containing an acid group, may be neutralized in a conventional manner, by the salts of organic fatty acids of the present invention, or both. The second polymer component, which may be partially or fully neutralized, preferably comprises ionomeric copolymers and terpolymers, ionomer precursors, thermoplastics, polyamides, polycarbonates, polyesters, polyurethanes, polyureas, thermoplastic elastomers, polybutadiene rubber, balata, metallocene-catalyzed polymers (grafted and non-grafted), single-site polymers, high-crystalline acid polymers, cationic ionomers, and the like.

The acid copolymers can be described as E/X/Y copolymers where E is ethylene, X is an  $\alpha,\beta$ -ethylenically unsaturated carboxylic acid, and Y is a softening comonomer. In a preferred embodiment, X is acrylic or methacrylic acid and Y is a  $C_{1-8}$  alkyl acrylate or methacrylate ester. X is preferably present in an amount from about 1 to about 35 weight percent of the polymer, more preferably from about 5 to about 30 weight percent of the polymer, and most preferably from about 10 to about 20 weight percent of the polymer. Y is preferably present in an amount from about 0 to about 50 weight percent of the polymer, more preferably from about 5 to about 25 weight percent of the polymer, and most preferably from about 10 to about 20 weight percent of the polymer.

The organic acids are aliphatic, mono-functional (saturated, unsaturated, or multi-unsaturated) organic acids. Salts of these organic acids may also be employed. The salts of organic acids of the present invention include the salts of barium, lithium, sodium, zinc, bismuth, chromium, cobalt, copper, potassium, strontium, titanium, tungsten, magnesium, cesium, iron, nickel, silver, aluminum, tin, or calcium, salts of fatty acids, particularly stearic, behenic, erucic, oleic, linoelic or dimerized derivatives thereof. It is preferred that the organic acids and salts of the present invention be relatively non-migratory (they do not bloom to the surface of the polymer under ambient temperatures) and non-volatile (they do not volatilize at temperatures required for melt-blending).

Thermoplastic polymer components, such as copolyetheresters, copolyesteresters, copolyetheramides, elastomeric polyolefins, styrene diene block copolymers and their hydrogenated derivatives, copolyesteramides, thermoplastic polyurethanes, such as copolyetherurethanes, copolyesterurethanes, copolyureaurethanes, epoxy-based polyurethanes, polycaprolactone-based polyurethanes, polyureas, and polycarbonate-based polyurethanes fillers, and other ingredients,

if included, can be blended in either before, during, or after the acid moieties are neutralized, thermoplastic polyurethanes.

Examples of these materials are disclosed in U.S. patent application Publication Nos. 2001/0018375 and 2001/0019971, which are incorporated herein, in their entirety, by express reference thereto.

U.S. application Ser. No. 10/230,015, now U.S. Publication No. 2003/0114565, and U.S. application Ser. No. 10/108,793, now U.S. Publication No. 2003/0050373, which are incorporated by reference herein in their entirety, discuss soft, highly resilient ionomers, which are preferably from neutralizing the acid copolymer(s) of at least one E/X/Y copolymer, where E is ethylene, X is the  $\alpha,\beta$ -ethylenically unsaturated carboxylic acid, and Y is a softening co-monomer. X is preferably present in 2-30 (preferably 4-20, most preferably 5-15) wt. % of the polymer, and Y is preferably present in 17-40 (preferably 20-40, and more preferably 24-35) wt. % of the polymer. Preferably, the melt index (MI) of the base resin is at least 20, or at least 40, more preferably, at least 75 and most preferably at least 150. Particular soft, resilient ionomers included in this invention are partially neutralized ethylene/(meth) acrylic acid/butyl (meth) acrylate copolymers having an MI and level of neutralization that results in a melt processible polymer that has useful physical properties. The copolymers are at least partially neutralized. Preferably at least 40, or, more preferably at least 55, even more preferably about 70, and most preferably about 80 of the acid moiety of the acid copolymer is neutralized by one or more alkali metal, transition metal, or alkaline earth metal cations. Cations useful in making the ionomers of this invention comprise lithium, sodium, potassium, magnesium, calcium, barium, or zinc, or a combination of such cations.

The invention also relates to a "modified" soft, resilient thermoplastic ionomer that comprises a melt blend of (a) the acid copolymers or the melt processible ionomers made therefrom as described above and (b) one or more organic acid(s) or salt(s) thereof, wherein greater than 80%, preferably greater than 90% of all the acid of (a) and of (b) is neutralized. Preferably, 100% of all the acid of (a) and (b) is neutralized by a cation source. Preferably, an amount of cation source in excess of the amount required to neutralize 100% of the acid in (a) and (b) is used to neutralize the acid in (a) and (b). Blends with fatty acids or fatty acid salts are preferred.

The organic acids or salts thereof are added in an amount sufficient to enhance the resilience of the copolymer. Preferably, the organic acids or salts thereof are added in an amount sufficient to substantially remove remaining ethylene crystallinity of the copolymer.

Preferably, the organic acids or salts are added in an amount of at least about 5% (weight basis) of the total amount of copolymer and organic acid(s). More preferably, the organic acids or salts thereof are added in an amount of at least about 15%, even more preferably at least about 20%. Preferably, the organic acid(s) are added in an amount up to about 50% (weight basis) based on the total amount of copolymer and organic acid. More preferably, the organic acids or salts thereof are added in an amount of up to about 40%, more preferably, up to about 35%. The non-volatile, non-migratory organic acids preferably are one or more aliphatic, mono-functional organic acids or salts thereof as described below, particularly one or more aliphatic, mono-functional, saturated or unsaturated organic acids having

## 11

less than 36 carbon atoms or salts of the organic acids, preferably stearic acid or oleic acid. Fatty acids or fatty acid salts are most preferred.

Processes for fatty acid (salt) modifications are known in the art. Particularly, the modified highly-neutralized soft, resilient acid copolymer ionomers of this invention can be produced by:

(a) melt-blending (1) ethylene,  $\alpha,\beta$ -ethylenically unsaturated  $C_{3-8}$  carboxylic acid copolymer(s) or melt-processible ionomer(s) thereof that have their crystallinity disrupted by addition of a softening monomer or other means with (2) sufficient non-volatile, non-migratory organic acids to substantially enhance the resilience and to disrupt (preferably remove) the remaining ethylene crystallinity, and then concurrently or subsequently

(b) Adding a sufficient amount of a cation source to increase the level of neutralization of all the acid moieties (including those in the acid copolymer and in the organic acid if the non-volatile, non-migratory organic acid is an organic acid) to the desired level.

The weight ratio of X to Y in the composition is at least about 1:20. Preferably, the weight ratio of X to Y is at least about 1:15, more preferably, at least about 1:10. Furthermore, the weight ratio of X to Y is up to about 1:1.67, more preferably up to about 1:2. Most preferably, the weight ratio of X to Y in the composition is up to about 1:2.2.

The acid copolymers used in the present invention to make the ionomers are preferably 'direct' acid copolymers (containing high levels of softening monomers). As noted above, the copolymers are at least partially neutralized, preferably at least about 40% of X in the composition is neutralized. More preferably, at least about 55% of X is neutralized. Even more preferably, at least about 70, and most preferably, at least about 80% of X is neutralized. In the event that the copolymer is highly neutralized (e.g., to at least 45%, preferably 50%, 55%, 70%, or 80%, of acid moiety), the MI of the acid copolymer should be sufficiently high so that the resulting neutralized resin has a measurable MI in accord with ASTM D-1238, condition E, at 190° C., using a 2160 gram weight. Preferably this resulting MI will be at least 0.1, preferably at least 0.5, and more preferably 1.0 or greater. Preferably, for highly neutralized acid copolymer, the MI of the acid copolymer base resin is at least 20, or at least 40, at least 75, and more preferably at least 150.

The acid copolymers preferably comprise alpha olefin, particularly ethylene,  $C_{3-8}$   $\alpha,\beta$ -ethylenically unsaturated carboxylic acid, particularly acrylic and methacrylic acid, and softening monomers, selected from alkyl acrylate, and alkyl methacrylate, wherein the alkyl groups have from 1-8 carbon atoms, copolymers. By "softening," it is meant that the crystallinity is disrupted (the polymer is made less crystalline). While the alpha olefin can be a  $C_2-C_4$  alpha olefin, ethylene is most preferred for use in the present invention. Accordingly, it is described and illustrated herein in terms of ethylene as the alpha olefin.

The acid copolymers, when the alpha olefin is ethylene, can be described as E/X/Y copolymers where E is ethylene, X is the  $\alpha,\beta$ -ethylenically unsaturated carboxylic acid, and Y is a softening co-monomer X is preferably present in 2-30 (preferably 4-20, most preferably 5-15) wt. % of the polymer, and Y is preferably present in 17-40 (preferably 20-40, most preferably 24-35) wt. % of the polymer.

The ethylene-acid copolymers with high levels of acid (X) are difficult to prepare in continuous polymerizers because of monomer-polymer phase separation. This difficulty can be avoided however by use of "co-solvent technology" as described in U.S. Pat. No. 5,028,674, or by employing

## 12

somewhat higher pressures than those which copolymers with lower acid can be prepared.

Specific acid-copolymers include ethylene/(meth) acrylic acid/n-butyl (meth) acrylate, ethylene/(meth) acrylic acid/iso-butyl (meth) acrylate, ethylene/(meth) acrylic acid/methyl (meth) acrylate, and ethylene/(meth) acrylic acid/ethyl (meth) acrylate terpolymers.

The organic acids employed are aliphatic, mono-functional (saturated, unsaturated, or multi-unsaturated) organic acids, particularly those having fewer than 36 carbon atoms. Also salts of these organic acids may be employed. Fatty acids or fatty acid salts are preferred. The salts may be any of a wide variety, particularly including the barium, lithium, sodium, zinc, bismuth, potassium, strontium, magnesium or calcium salts of the organic acids. Particular organic acids useful in the present invention include caproic acid, caprylic acid, capric acid, lauric acid, stearic acid, behenic acid, erucic acid, oleic acid, and linoleic acid.

The optional filler component is chosen to impart additional density to blends of the previously described components, the selection being dependent upon the different parts (e.g., cover, mantle, core, center, intermediate layers in a multilayered core or ball) and the type of golf ball desired (e.g., one-piece, two-piece, three-piece or multiple-piece ball), as will be more fully detailed below.

Generally, the filler will be inorganic having a density greater than about 4 grams/cubic centimeter ( $g/cm^3$ ), preferably greater than 5  $g/cm^3$ , and will be present in amounts between 0 to about 60 wt. % based on the total weight of the composition. Examples of useful fillers include zinc oxide, barium sulfate, lead silicate and tungsten carbide, as well as the other well-known fillers used in golf balls. It is preferred that the filler materials be non-reactive or almost non-reactive and not stiffen or raise the compression nor reduce the coefficient of restitution significantly.

Additional optional additives useful in the practice of the subject invention include acid copolymer wax (e.g., Allied wax AC 143 believed to be an ethylene/16-18% acrylic acid copolymer with a number average molecular weight of 2,040), which assist in preventing reaction between the filler materials (e.g.,  $ZnO$ ) and the acid moiety in the ethylene copolymer. Other optional additives include  $TiO_2$ , which is used as a whitening agent; optical brighteners; surfactants; processing aids; etc.

Ionomers may be blended with conventional ionomeric copolymers (di-, ter-, etc.), using well-known techniques, to manipulate product properties as desired. The blends would still exhibit lower hardness and higher resilience when compared with blends based on conventional ionomers.

Also, ionomers can be blended with non-ionic thermoplastic resins to manipulate product properties. The non-ionic thermoplastic resins would, by way of non-limiting illustrative examples, include thermoplastic elastomers, such as polyurethane, poly-ether-ester, poly-amide-ether, polyether-urea, PEBA<sup>®</sup> (a family of block copolymers based on polyether-block-amide, commercially supplied by Atochem), styrene-butadiene-styrene (SBS) block copolymers, styrene(ethylene-butylene)-styrene block copolymers, etc., poly amide (oligomeric and polymeric), polyesters, polyolefins including PE, PP, E/P copolymers, etc., ethylene copolymers with various comonomers, such as vinyl acetate, (meth)acrylates, (meth)acrylic acid, epoxy-functionalized monomer, CO, etc., functionalized polymers with maleic anhydride grafting, epoxidization etc., elastomers, such as EPDM, metallocene catalyzed PE and copolymer, ground up powders of the thermoset elastomers, etc. Such thermoplas-

## 13

tic blends comprise about 1% to about 99% by weight of a first thermoplastic and about 99% to about 1% by weight of a second thermoplastic.

Additionally, the compositions of U.S. application Ser. No. 10/269,341, now U.S. Publication No. 20030130434, and U.S. Pat. No. 6,653,382, both of which are incorporated herein in their entirety, discuss compositions having high COR when formed into solid spheres.

The thermoplastic composition of this invention comprises a polymer which, when formed into a sphere that is 1.50 to 1.54 inches in diameter, has a coefficient of restitution (COR) when measured by firing the sphere at an initial velocity of 125 feet/second against a steel plate positioned 3 feet from the point where initial velocity and rebound velocity are determined and by dividing the rebound velocity from the plate by the initial velocity and an Atti compression of no more than 100.

The thermoplastic composition of this invention preferably comprises (a) aliphatic, mono-functional organic acid(s) having fewer than 36 carbon atoms; and (b) ethylene,  $C_3$  to  $C_8$   $\alpha,\beta$ -ethylenically unsaturated carboxylic acid copolymer(s) and ionomer(s) thereof, wherein greater than 90%, preferably near 100%, and more preferably 100% of all the acid of (a) and (b) are neutralized.

The thermoplastic composition preferably comprises melt-processible, highly-neutralized (greater than 90%, preferably near 100%, and more preferably 100%) polymer of (1) ethylene,  $C_3$  to  $C_8$   $\alpha,\beta$ -ethylenically unsaturated carboxylic acid copolymers that have their crystallinity disrupted by addition of a softening monomer or other means such as high acid levels, and (2) non-volatile, non-migratory agents such as organic acids (or salts) selected for their ability to substantially or totally suppress any remaining ethylene crystallinity. Agents other than organic acids (or salts) may be used.

It has been found that, by modifying an acid copolymer or ionomer with a sufficient amount of specific organic acids (or salts thereof); it is possible to highly neutralize the acid copolymer without losing processability or properties such as elongation and toughness. The organic acids employed in the present invention are aliphatic, mono-functional, saturated or unsaturated organic acids, particularly those having fewer than 36 carbon atoms, and particularly those that are non-volatile and non-migratory and exhibit ionic array plasticizing and ethylene crystallinity suppression properties.

With the addition of sufficient organic acid, greater than 90%, nearly 100%, and preferably 100% of the acid moieties in the acid copolymer from which the ionomer is made can be neutralized without losing the processability and properties of elongation and toughness.

The melt-processible, highly-neutralized acid copolymer ionomer can be produced by the following:

(a) melt-blending (1) ethylene  $\alpha,\beta$ -ethylenically unsaturated  $C_{3-8}$  carboxylic acid copolymer(s) or melt-processible ionomer(s) thereof (ionomers that are not neutralized to the level that they have become intractable, that is not melt-processible) with (1) one or more aliphatic, mono-functional, saturated or unsaturated organic acids having fewer than 36 carbon atoms or salts of the organic acids, and then concurrently or subsequently

(b) Adding a sufficient amount of a cation source to increase the level of neutralization all the acid moieties (including those in the acid copolymer and in the organic acid) to greater than 90%, preferably near 100%, more preferably to 100%.

Preferably, highly-neutralized thermoplastics of the invention can be made by:

## 14

(a) melt-blending (1) ethylene,  $\alpha,\beta$ -ethylenically unsaturated  $C_{3-8}$  carboxylic acid copolymer(s) or melt-processible ionomer(s) thereof that have their crystallinity disrupted by addition of a softening monomer or other means with (2) sufficient non-volatile, non-migratory agents to substantially remove the remaining ethylene crystallinity, and then concurrently or subsequently

(b) adding a sufficient amount of a cation source to increase the level of neutralization all the acid moieties (including those in the acid copolymer and in the organic acid if the non-volatile, non-migratory agent is an organic acid) to greater than 90%, preferably near 100%, more preferably to 100%.

The acid copolymers used in the present invention to make the ionomers are preferably 'direct' acid copolymers. They are preferably alpha olefin, particularly ethylene,  $C_{3-8}$   $\alpha,\beta$ -ethylenically unsaturated carboxylic acid, particularly acrylic and methacrylic acid, copolymers. They may optionally contain a third softening monomer. By "softening," it is meant that the crystallinity is disrupted (the polymer is made less crystalline). Suitable "softening" co-monomers are monomers selected from alkyl acrylate, and alkyl methacrylate, wherein the alkyl groups have from 1-8 carbon atoms.

The acid copolymers, when the alpha olefin is ethylene, can be described as E/X/Y copolymers where E is ethylene, X is the  $\alpha,\beta$ -ethylenically unsaturated carboxylic acid, and Y is a softening comonomer. X is preferably present in 3-30 (preferably 4-25, most preferably 5-20) wt. % of the polymer, and Y is preferably present in 0-30 (alternatively 3-25 or 10-23) wt. % of the polymer. Spheres were prepared using fully neutralized ionomers A and B as presented in Table I.

TABLE I

| 40 | Sample | Resin Type (%) | Acid Type (%) | Cation    |                 |
|----|--------|----------------|---------------|-----------|-----------------|
|    |        |                |               | (% neut*) | M.I. (g/10 min) |
|    | 1A     | A (60)         | Oleic (40)    | Mg (100)  | 1.0             |
|    | 2B     | A (60)         | Oleic (40)    | Mg (105)* | 0.9             |
|    | 3C     | B (60)         | Oleic (40)    | Mg (100)  | 0.9             |
| 45 | 4D     | B (60)         | Oleic (40)    | Mg (105)* | 0.9             |
|    | 5E     | B (60)         | Stearic (40)  | Mg (100)  | 0.85            |

A - ethylene, 14.8% normal butyl acrylate, 8.3% acrylic acid

B - ethylene, 14.9% normal butyl acrylate, 10.1% acrylic acid

50 \*indicates that cation was sufficient to neutralize 105% of all the acid in the resin and the organic acid.

These compositions were molded into 1.53-inch spheres for which data is presented in the following table.

TABLE II

| 55 | Sample | Atti Compression | COR @ 125 ft/s |  |
|----|--------|------------------|----------------|--|
|    |        |                  |                |  |
|    | 1A     | 75               | 0.826          |  |
|    | 2B     | 75               | 0.826          |  |
|    | 3C     | 78               | 0.837          |  |
|    | 4D     | 76               | 0.837          |  |
|    | 5E     | 97               | 0.807          |  |

65 Further testing of commercially available highly neutralized polymers HNP1 and HNP2 had the following properties.

TABLE III

| Material Properties            |        | HNP1   | HNP2  |
|--------------------------------|--------|--------|-------|
| Specific Gravity               |        | 0.966  | 0.974 |
| Melt Flow, 190° C., 10-kg load |        | 0.65   | 1.0   |
| Shore D Flex Bar (40 hr)       |        | 47.0   | 46.0  |
| Shore D Flex Bar (2 week)      |        | 51.0   | 48.0  |
| Flex Modulus, psi (40 hr)      | 25,800 | 16,100 |       |
| Flex Modulus, psi (2 week)     | 39,900 | 21,000 |       |
| DSC Melting Point (° C.)       | 61.0   | 61/101 |       |
| Moisture (ppm)                 | 1500   | 4500   |       |
| Weight % Mg                    | 2.65   | 2.96   |       |

TABLE IV

| Material    | Solid Sphere Data |       |          |          |                              |
|-------------|-------------------|-------|----------|----------|------------------------------|
|             | HNP1              | HNP2  | HNP2a    | HNP1a    | HNP1a/HNP2a<br>(50:50 blend) |
| Spec. Grav. | 0.954             | 0.959 | 1.153    | 1.146    | 1.148                        |
| Filler      | None              | None  | Tungsten | Tungsten | Tungsten                     |
| Compression | 107               | 83    | 86       | 62       | 72                           |
| COR         | 0.827             | 0.853 | 0.844    | 0.806    | 0.822                        |
| Shore D     | 51                | 47    | 49       | 42       | 45                           |
| Shore C     |                   |       | 79       | 72       | 75                           |

These materials are exemplary examples of the preferred center and/or core layer compositions of the present invention. They may also be used as a cover layer herein.

While the outer cover may be formed of any of the above-listed materials, the outer cover preferably includes a polyurethane, polyurea, or epoxy composition, generally comprising the reaction product of at least one polyisocyanate, polyol, and at least one curing agent. Any polyisocyanate available to one of ordinary skill in the art is suitable for use according to the invention. Exemplary polyisocyanates include, but are not limited to, 4,4'-diphenylmethane diisocyanate ("MDI"); polymeric MDI; carbodiimide-modified liquid MDI; 4,4'-dicyclohexylmethane diisocyanate ("H<sub>12</sub>MDI"); p-phenylene diisocyanate ("PPDI"); m-phenylene diisocyanate ("MPDI"); toluene diisocyanate ("TDI"); 3,3'-dimethyl-4,4'-biphenylene diisocyanate ("TODI"); isophorone diisocyanate ("IPDI"); hexamethylene diisocyanate ("HDI"); naphthalene diisocyanate ("NDI"); xylene diisocyanate ("XDI"); p-tetramethylxylene diisocyanate ("p-TMXDI"); m-tetramethylxylene diisocyanate ("m-TMXDI"); ethylene diisocyanate; propylene-1,2-diisocyanate; tetramethylene-1,4-diisocyanate; cyclohexyl diisocyanate; 1,6-hexamethylene-diisocyanate ("HDI"); dodecane-1,12-diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; methyl cyclohexylene diisocyanate; triisocyanate of HDI; triisocyanate of 2,4,4-trimethyl-1,6-hexane diisocyanate ("TMDI"); tetracene diisocyanate; naphthalene diisocyanate; anthracene diisocyanate; isocyanurate of toluene diisocyanate; uretdione of hexamethylene diisocyanate; and mixtures thereof. Preferably, the polyisocyanate includes MDI, PPDI, TDI, or a mixture thereof, and more preferably, the polyisocyanate includes MDI. It should be understood that, as used herein, the term "MDI" includes 4,4'-diphenylmethane diisocyanate, polymeric MDI, carbodiimide-modified liquid MDI, and mixtures thereof and, additionally, that the diisocyanate employed may be "low free monomer," understood by one of ordinary skill in the art to have lower

levels of "free" monomer isocyanate groups, typically less than about 0.1% free monomer groups. Examples of "low free monomer" diisocyanates include, but are not limited to Low Free Monomer MDI, Low Free Monomer TDI, and Low Free Monomer PPDI.

The at least one polyisocyanate should have less than about 14% unreacted NCO groups. Preferably, the at least one polyisocyanate has no greater than about 7.5% NCO, and more preferably, less than about 7.0%.

10 Any polyol available to one of ordinary skill in the art is suitable for use according to the invention. Exemplary polyols include, but are not limited to, polyether polyols, hydroxy-terminated polybutadiene (including partially/fully hydrogenated derivatives), polyester polyols, polycaprolactone polyols, and polycarbonate polyols. In one preferred embodiment, the polyol includes polyether polyol. Examples include, but are not limited to, polytetramethylene ether glycol ("PTMEG"), polyethylene propylene glycol,

15 polyoxypropylene glycol, and mixtures thereof. The hydrocarbon chain can have saturated or unsaturated bonds and substituted or unsubstituted aromatic and cyclic groups. Preferably, the polyol of the present invention includes PTMEG.

20 Suitable polyester polyols include, but are not limited to, polyethylene adipate glycol; polybutylene adipate glycol; polyethylene propylene adipate glycol; o-phthalate-1,6-hexanediol; poly(hexamethylene adipate) glycol; and mixtures thereof. The hydrocarbon chain can have saturated or unsaturated bonds, or substituted or unsubstituted aromatic and cyclic groups.

25 Suitable polycaprolactone polyols include, but are not limited to, 1,6-hexanediol-initiated polycaprolactone, diethylene glycol initiated polycaprolactone, trimethylol propane initiated polycaprolactone, neopentyl glycol initiated polycaprolactone, 1,4-butanediol-initiated polycaprolactone, PTMEG-initiated polycaprolactone, and mixtures thereof. The hydrocarbon chain can have saturated or unsaturated bonds, or substituted or unsubstituted aromatic and cyclic groups.

30 Suitable polycarbonates include, but are not limited to, polyphthalate carbonate and poly(hexamethylene carbonate) glycol. The hydrocarbon chain can have saturated or unsaturated bonds, or substituted or unsubstituted aromatic and cyclic groups.

35 Suitable polyamine curatives are also suitable for use in polyurethane covers. Preferred polyamine curatives include, but are not limited to, 3,5-dimethylthio-2,4-toluenediamine and isomers thereof; 3,5-diethyltoluene-2,4-diamine and isomers thereof, such as 3,5-diethyltoluene-2,6-diamine; 4,4'-bis(sec-butylamino)-diphenylmethane; 1,4-bis(sec-butylamino)-benzene, 4,4'-methylene-bis-(2-chloroaniline); 4,4'-methylene-bis-(3-chloro-2,6-diethylaniline) ("MCDEA"); polytetramethyleneoxide-di-p-aminobenzoate; N,N'-dialkyldiamino diphenyl methane; p,p'-methylene dianiline ("MDA"); m-phenylenediamine ("MPDA"); 4,4'-methylene-bis-(2-chloroaniline) ("MOCA"); 4,4'-methylene-bis-(2,6-diethylaniline) ("MDEA"); 4,4'-methylene-bis-(2,3-dichloroaniline) ("MDCA"); 4,4'-diamino-3,3'-diethyl-5,5'-dimethyl diphenylmethane; 2,2',3,3'-tetrachloro diamino diphenylmethane; trimethylene glycol di-p-aminobenzoate; and mixtures thereof. Preferably, the curing agent of the present invention includes 3,5-dimethylthio-2,4-toluenediamine and isomers thereof, such as Ethacure® 300, commercially available from Albermarle Corporation of Baton Rouge, La. Suitable polyamine curatives include both primary and secondary amines.

At least one of a diol, triol, tetraol, or hydroxy-terminated curatives may be added to the aforementioned polyurethane composition. Suitable diol, triol, and tetraol groups include ethylene glycol; diethylene glycol; polyethylene glycol; propylene glycol; polypropylene glycol; lower molecular weight polytetramethylene ether glycol; 1,3-bis(2-hydroxyethoxy) benzene; 1,3-bis-[2-(2-hydroxyethoxy) ethoxy]benzene; 1,3-bis-{2-[2-(2-hydroxyethoxy) ethoxy]ethoxy}benzene; 1,4-butanediol; 1,5-pentanediol; 1,6-hexanediol; resorcinol-di-( $\beta$ -hydroxyethyl) ether; hydroquinone-di-( $\beta$ -hydroxyethyl) ether; and mixtures thereof. Preferred hydroxy-terminated curatives include 1,3-bis(2-hydroxyethoxy) benzene; 1,3-bis-[2-(2-hydroxyethoxy) ethoxy]benzene; 1,3-bis-{2-[2-(2-hydroxyethoxy) ethoxy]ethoxy}benzene; 1,4-butanediol, and mixtures thereof.

Both the hydroxy-terminated and amine curatives can include one or more saturated, unsaturated, aromatic, and cyclic groups. Additionally, the hydroxy-terminated and amine curatives can include one or more halogen groups. The polyurethane composition can be formed with a blend or mixture of curing agents. If desired, however, the polyurethane composition may be formed with a single curing agent.

In a particularly preferred embodiment of the present invention, saturated polyurethanes used to form cover layers, preferably the outer cover layer, and may be selected from among both castable thermoset and thermoplastic polyurethanes. In this embodiment, the saturated polyurethanes are substantially free of aromatic groups or moieties.

Saturated diisocyanates which can be used include, but are not limited to, ethylene diisocyanate; propylene-1,2-diisocyanate; tetramethylene-1,4-diisocyanate; 1,6-hexamethylene-diisocyanate ("HDI"); 2,2,4-trimethylhexamethylene diisocyanate; 2,4,4-trimethylhexamethylene diisocyanate; dodecane-1,12-diisocyanate; dicyclohexylmethane diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; isophorone diisocyanate ("IPDI"); methyl cyclohexylene diisocyanate; triisocyanate of HDI; triisocyanate of 2,2,4-trimethyl-1,6-hexane diisocyanate ("TMDI"). The most preferred saturated diisocyanates are 4,4'-dicyclohexylmethane diisocyanate ("HMDI") and isophorone diisocyanate ("IPDI").

Saturated polyols which are appropriate for use in this invention include, but are not limited to, polyether polyols such as polytetramethylene ether glycol and poly(oxypropylene) glycol. Suitable saturated polyester polyols include polyethylene adipate glycol, polyethylene propylene adipate glycol, polybutylene adipate glycol, polycarbonate polyol and ethylene oxide-capped polyoxypropylene diols. Saturated polycaprolactone polyols which are useful in the invention include diethylene glycol initiated polycaprolactone, 1,4-butanediol initiated polycaprolactone, 1,6-hexanediol initiated polycaprolactone; trimethylol propane initiated polycaprolactone, neopentyl glycol initiated polycaprolactone, PTMEG-initiated polycaprolactone. The most preferred saturated polyols are PTMEG and PTMEG-initiated polycaprolactone.

Suitable saturated curatives include 1,4-butanediol, ethylene glycol, diethylene glycol, polytetramethylene ether glycol, propylene glycol; trimethanolpropane; tetra-(2-hydroxypropyl)-ethylenediamine; isomers and mixtures of isomers of cyclohexyldimethylol, isomers and mixtures of isomers of cyclohexane bis(methylamine); triisopropanolamine, ethylene diamine, diethylene triamine, triethylene

tetramine, tetraethylene pentamine, 4,4'-dicyclohexylmethane diamine, 2,2,4-trimethyl-1,6-hexanediamine; 2,4,4-trimethyl-1,6-hexanediamine; diethyleneglycol di-(aminopropyl)ether; 4,4'-bis-(sec-butylamino)-dicyclohexylmethane; 1,2-bis-(sec-butylamino)cyclohexane; 1,4-bis-(sec-butylamino)cyclohexane; isophorone diamine, hexamethylene diaamine, propylene diamine, 1-methyl-2,4-cyclohexyl diamine, 1-methyl-2,6-cyclohexyl diamine, 1,3-diaminopropane, dimethylamino propylamine, diethylamino propylamine, imido-bis-propylamine, isomers and mixtures of isomers of diaminocyclohexane, monoethanolamine, diethanolamine, triethanolamine, monoisopropanolamine, and diisopropanolamine. The most preferred saturated curatives are 1,4-butanediol, 1,4-cyclohexyldimethylol and 4,4'-bis-(sec-butylamino)-dicyclohexylmethane.

Suitable catalysts include, but are not limited to bismuth catalyst, oleic acid, triethylenediamine (DABCO®-33LV), di-butyltin dilaurate (DABCO®-T12) and acetic acid. The most preferred catalyst is di-butyltin dilaurate (DABCO®-T12). DABCO® materials are manufactured by Air Products and Chemicals, Inc.

It is well known in the art that if the saturated polyurethane materials are to be blended with other thermoplastics, care must be taken in the formulation process so as to produce an end product which is thermoplastic in nature. Thermoplastic materials may be blended with other thermoplastic materials, but thermosetting materials are difficult if not impossible to blend homogeneously after the thermosetting materials are formed. Preferably, the saturated polyurethane comprises from about 1 to about 100%, more preferably from about 10 to about 75% of the cover composition and/or the intermediate layer composition. About 90 to about 10%, more preferably from about 90 to about 25% of the cover and/or the intermediate layer composition is comprised of one or more other polymers and/or other materials as described below. Such polymers include, but are not limited to polyurethane/polyurea ionomers, polyurethanes or polyureas, epoxy resins, polyethylenes, polyamides and polyesters, polycarbonates and polyacrylin. Unless otherwise stated herein, all percentages are given in percent by weight of the total composition of the golf ball layer in question.

Polyurethane prepolymers are produced by combining at least one polyol, such as a polyether, polycaprolactone, polycarbonate or a polyester, and at least one isocyanate. Thermosetting polyurethanes are obtained by curing at least one polyurethane prepolymer with a curing agent selected from a polyamine, triol or tetraol. Thermoplastic polyurethanes are obtained by curing at least one polyurethane prepolymer with a diol curing agent. The choice of the curatives is critical because some urethane elastomers that are cured with a diol and/or blends of diols do not produce urethane elastomers with the impact resistance required in a golf ball cover. Blending the polyamine curatives with diol cured urethane elastomeric formulations leads to the production of thermoset urethanes with improved impact and cut resistance.

Thermoplastic polyurethanes may be blended with suitable materials to produce a thermoplastic end product. Examples of such additional materials may include ionomers such as the SURLYN®, ESCOR® and IOTEK® copolymers described above.

Other suitable materials which may be combined with the saturated polyurethanes in forming the cover and/or intermediate layer(s) of the golf balls of the invention include ionic or non-ionic polyurethanes and polyureas, epoxy res-

ins, polyethylenes, polyamides and polyesters. For example, the cover and/or intermediate layer may be formed from a blend of at least one saturated polyurethane and thermoplastic or thermoset ionic and non-ionic urethanes and polyurethanes, cationic urethane ionomers and urethane epoxies, ionic and non-ionic polyureas and blends thereof. Examples of suitable urethane ionomers are disclosed in U.S. Pat. No. 5,692,974 entitled "Golf Ball Covers," the disclosure of which is hereby incorporated by reference in its entirety. Other examples of suitable polyurethanes are described in U.S. Pat. No. 5,334,673. Examples of appropriate polyureas are discussed in U.S. Pat. No. 5,484,870 and examples of suitable polyurethanes cured with epoxy group containing curing agents are disclosed in U.S. Pat. No. 5,908,358, the disclosures of which are hereby incorporated herein by reference in their entirety.

A variety of conventional components can be added to the cover compositions of the present invention. These include, but are not limited to, white pigment such as  $TiO_2$ ,  $ZnO$ , optical brighteners, surfactants, processing aids, foaming agents, density-controlling fillers, UV stabilizers and light stabilizers. Saturated polyurethanes are resistant to discoloration. However, they are not immune to deterioration in their mechanical properties upon weathering. Addition of UV absorbers and light stabilizers to any of the above compositions and, in particular, the polyurethane compositions, help to maintain the tensile strength, elongation, and color stability. Suitable UV absorbers and light stabilizers include TINUVIN® 328, TINUVIN® 213, TINUVIN® 765, TINUVIN® 770 and TINUVIN® 622. The preferred UV absorber is TINUVIN® 328, and the preferred light stabilizer is TINUVIN® 765. TINUVIN® products are available from Ciba-Geigy. Dyes, as well as optical brighteners and fluorescent pigments may also be included in the golf ball covers produced with polymers formed according to the present invention. Such additional ingredients may be added in any amounts that will achieve their desired purpose.

Any method known to one of ordinary skill in the art may be used to polyurethanes of the present invention. One commonly employed method, known in the art as a one-shot method, involves concurrent mixing of the polyisocyanate, polyol, and curing agent. This method results in a mixture that is inhomogenous (more random) and affords the manufacturer less control over the molecular structure of the resultant composition. A preferred method of mixing is known as a prepolymer method. In this method, the polyisocyanate and the polyol are mixed separately prior to addition of the curing agent. This method affords a more homogeneous mixture resulting in a more consistent polymer composition. Other methods suitable for forming the layers of the present invention include reaction injection molding ("RIM"), liquid injection molding ("LIM"), and pre-reacting the components to form an injection moldable thermoplastic polyurethane and then injection molding, all of which are known to one of ordinary skill in the art.

It has been found by the present invention that the use of a castable, reactive material, which is applied in a fluid form, makes it possible to obtain very thin outer cover layers on golf balls. Specifically, it has been found that castable, reactive liquids, which react to form a urethane elastomer material, provide desirable very thin outer cover layers.

The castable, reactive liquid employed to form the urethane elastomer material can be applied over the core using a variety of application techniques such as spraying, dipping, spin coating, or flow coating methods which are well known in the art. An example of a suitable coating technique

is that which is disclosed in U.S. Pat. No. 5,733,428, the disclosure of which is hereby incorporated by reference in its entirety in the present application.

The outer cover is preferably formed around the inner cover by mixing and introducing the material in the mold halves. It is important that the viscosity be measured over time, so that the subsequent steps of filling each mold half, introducing the core into one half and closing the mold can be properly timed for accomplishing centering of the core 5 cover halves fusion and achieving overall uniformity. Suitable viscosity range of the curing urethane mix for introducing cores into the mold halves is determined to be approximately between about 2,000 cP and about 30,000 cP, with the preferred range of about 8,000 cP to about 15,000 cP.

To start the cover formation, mixing of the prepolymer and curative is accomplished in motorized mixer including mixing head by feeding through lines metered amounts of curative and prepolymer. Top preheated mold halves are 10 filled and placed in fixture units using centering pins moving into holes in each mold. At a later time, a bottom mold half or a series of bottom mold halves have similar mixture amounts introduced into the cavity. After the reacting materials have resided in top mold halves for about 40 to about 15 20 seconds, a core is lowered at a controlled speed into the gelling reacting mixture.

A ball cup holds the ball core through reduced pressure (or partial vacuum). Upon location of the coated core in the 25 halves of the mold after gelling for about 40 to about 80 seconds, the vacuum is released allowing core to be 30 released. The mold halves, with core and solidified cover half thereon, are removed from the centering fixture unit, inverted and mated with other mold halves which, at an appropriate time earlier, have had a selected quantity of 35 reacting polyurethane prepolymer and curing agent introduced therein to commence gelling.

Similarly, U.S. Pat. Nos. 5,006,297 and 5,334,673 both 40 also disclose suitable molding techniques which may be utilized to apply the castable reactive liquids employed in the present invention. Further, U.S. Pat. Nos. 6,180,040 and 6,180,722 disclose methods of preparing dual core golf 45 balls. The disclosures of these patents are hereby incorporated by reference in their entirety. However, the method of the invention is not limited to the use of these techniques.

The molding process and composition of golf ball portions typically results in a gradient of material properties. Methods employed in the prior art generally exploit hardness to quantify these gradients. Hardness is a qualitative 50 measure of static modulus and does not represent the modulus of the material at the deformation rates associated with golf ball use, i.e., impact by a club. As is well known to one skilled in the art of polymer science, the time-temperature superposition principle may be used to emulate alternative deformation rates. For golf ball portions including polybutadiene, a 1-Hz oscillation at temperatures between 0° C. and -50° C. are believed to be qualitatively equivalent to golf ball impact rates. Therefore, measurement of loss tangent and dynamic stiffness at 0° C. to -50° C. may be used to accurately anticipate golf ball performance, preferably at temperatures between about -20° C. and -50° C.

The resultant golf balls typically have a coefficient of 55 restitution of greater than about 0.7, preferably greater than about 0.75, and more preferably greater than about 0.78. The golf balls also typically have an Atti compression of at least about 40, preferably from about 50 to 120, and more preferably from about 60 to 100. The golf ball cured polybutadiene material typically has a hardness of at least

## 21

about 15 Shore A, preferably between about 30 Shore A and 80 Shore D, more preferably between about 50 Shore A and 60 Shore D.

When golf balls are prepared according to the invention, they typically will have dimple coverage greater than about 60 percent, preferably greater than about 65 percent, and more preferably greater than about 75 percent. The flexural modulus of the cover on the golf balls, as measured by ASTM method D6272-98, Procedure B, is typically greater than about 500 psi, and is preferably from about 500 psi to 150,000 psi. As discussed herein, the outer cover layer is preferably formed from a relatively soft polyurethane material. In particular, the material of the outer cover layer should have a material hardness, as measured by ASTM-D2240, less than about 45 Shore D, preferably less than about 40 Shore D, more preferably between about 25 and about 40 Shore D, and most preferably between about 30 and about 40 Shore D. Alternatively, the material of the outer cover layer should have a material hardness of less than about 60 Shore D, preferably less than about 55 Shore D, and more preferably between about 40 and about 55 Shore D. The casing preferably has a material hardness of less than about 70 Shore D, more preferably between about 30 and about 70 Shore D, and most preferably, between about 50 and about 65 Shore D.

It should be understood, especially to one of ordinary skill in the art, that there is a fundamental difference between "material hardness" and "hardness, as measured directly on a golf ball." Material hardness is defined by the procedure set forth in ASTM-D2240 and generally involves measuring the hardness of a flat "slab" or "button" formed of the material of which the hardness is to be measured. Hardness, when measured directly on a golf ball (or other spherical surface) is a completely different measurement and, therefore, results in a different hardness value. This difference results from a number of factors including, but not limited to, ball construction (i.e., core type, number of core and/or cover layers, etc.), ball (or sphere) diameter, and the material composition of adjacent layers. It should also be understood that the two measurement techniques are not linearly related and, therefore, one hardness value cannot easily be correlated to the other.

## 22

The core of the present invention has an Atti compression of less than about 80, more preferably, between about 40 and about 80, and most preferably, between about 50 and about 70. In an alternative, low compression embodiment, the core has a compression less than about 20, more preferably less than about 10, and most preferably, 0. The overall outer diameter ("OD") of the core is less than about 1.610 inches, preferably, no greater than 1.590 inches, more preferably between about 1.540 inches and about 1.580 inches, and most preferably between about 1.50 inches to about 1.570 inches. The OD of the casing of the golf balls of the present invention is preferably between 1.580 inches and about 1.640 inches, more preferably between about 1.590 inches to about 1.630 inches, and most preferably between about 1.600 inches to about 1.630 inches.

The present multilayer golf ball can have an overall diameter of any size. Although the United States Golf Association ("USGA") specifications limit the minimum size of a competition golf ball to 1.680 inches. There is no specification as to the maximum diameter. Golf balls of any size, however, can be used for recreational play. The preferred diameter of the present golf balls is from about 1.680 inches to about 1.800 inches. The more preferred diameter is from about 1.680 inches to about 1.760 inches. The most preferred diameter is about 1.680 inches to about 1.740 inches.

## EXAMPLES

35 Three solid cores, each having an outer diameter of 1.58 inches, were formed of a composition comprising polybutadiene rubber, zinc diacrylate, zinc oxide, dicumyl peroxide, barium sulfate, and color dispersion. One core, representative of conventional technology, was used as a control. The 40 two remaining cores were each additionally blended with 5.3 parts Struktol® A95 (Example 1) and the zinc salt of pentachlorothiophenol at 2.4 parts (Example 2). Struktol® A95 at 5.3 parts contains 2.4 parts PCTP. The specific compositions for each of the solid cores are presented below in Table I.

TABLE I

|                         | CONTROL |       |       |       | EXAMPLE 1 |       |       |       | EXAMPLE 2 |       |      |      |
|-------------------------|---------|-------|-------|-------|-----------|-------|-------|-------|-----------|-------|------|------|
| INGREDIENT              | 100     | 100   | 100   | 100   | 100       | 100   | 100   | 100   | 100       | 100   | 100  | 100  |
| polybutadiene rubber    | 100     | 100   | 100   | 100   | 100       | 100   | 100   | 100   | 100       | 100   | 100  | 100  |
| zinc diacrylate         | 18      | 25    | 30    | 27    | 34        | 41    | 20    | 25    | 30        | 35    |      |      |
| dicumyl peroxide        | 0.5     | 0.5   | 0.5   | 1.8   | 1.8       | 1.8   | 0.8   | 0.8   | 0.8       | 0.8   | 0.8  | 0.8  |
| Struktol® A95 PCTP      | —       | —     | —     | 5.3   | 5.3       | 5.3   | —     | —     | —         | —     | —    | —    |
| zinc salt of PCTP       | —       | —     | —     | —     | —         | —     | 2.4   | 2.4   | 2.4       | 2.4   | 2.4  | 2.4  |
| zinc oxide              | 26.5    | 24.1  | 22.2  | 5     | 5         | 5     | 5     | 5     | 5         | 5     | 5    | 5    |
| barium sulfate          | —       | —     | —     | 16.2  | 13.4      | 10.6  | 21.7  | 19.7  | 17.7      | 15.7  |      |      |
| color dispersion        | 0.14    | 0.14  | 0.14  | 0.14  | 0.14      | 0.14  | 0.14  | 0.14  | 0.14      | 0.14  | 0.14 | 0.14 |
| PROPERTY                |         |       |       |       |           |       |       |       |           |       |      |      |
| Effective Modulus (psi) | 3800    | 6200  | 8700  | 4100  | 6200      | 7700  | 3600  | 5100  | 7400      | 9700  |      |      |
| Atti Compression        | 17      | 52    | 76    | 22    | 52        | 67    | 13    | 38    | 65        | 84    |      |      |
| COR @ 125 ft/s          | 0.764   | 0.789 | 0.802 | 0.773 | 0.794     | 0.802 | 0.782 | 0.801 | 0.813     | 0.823 |      |      |

It is very apparent that the addition of PCTP, in either form, increases COR, decreases compression, or both. In particular, the PCTP zinc salt (Example 2) provides comparable COR's with lower compression and/or increased COR's with comparable (or lower) compression, both of which are desirable golf ball properties.

The halogenated organosulfur polymers of the present invention may also be used in golf equipment, in particular, inserts for golf clubs, such as putters, irons, and woods, and in golf shoes and components thereof.

As used herein, the term "about," used in connection with one or more numbers or numerical ranges, should be understood to refer to all such numbers, including all numbers in a range.

Other than in the operating examples, or unless otherwise expressly specified, all of the numerical ranges, amounts, values and percentages, such as those for amounts of materials and others, in the following portion of the specification may be read as if prefaced by the word "about" even though the term "about" may not expressly appear with the value, amount or range. Accordingly, unless indicated to the contrary, the numerical parameters set forth in the specification and attached claims are approximations that may vary depending upon the desired properties sought to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contain certain errors necessarily resulting from the standard deviation found in their respective testing measurements. Furthermore, when numerical ranges of varying scope are set forth herein, it is contemplated that any combination of these values inclusive of the recited values may be used.

While it is apparent that the illustrative embodiments of the invention disclosed herein fulfill the preferred embodiments of the present invention, it is appreciated that numerous modifications and other embodiments may be devised by those skilled in the art. Therefore, it will be understood that the appended claims are intended to cover all such modifications and embodiments, which would come within the spirit and scope of the present invention.

What is claimed is:

1. A golf ball comprising:  
a core having a diameter of between about 1.54 inches and about 1.57 inches, a compression of between about 70 and 80, and comprising a polybutadiene rubber composition comprising a magnesium salt of pentachlorothiophenol;  
a cover having a thickness of about 0.04 inches or less and comprising a castable polyurethane or polyurea composition; and  
an inner cover layer disposed between the core and the outer cover layer, the inner cover layer having a thickness of about 0.04 inches or less and selected from the group consisting of ionomers, vinyl resins, polyolefins, polyurethanes, polyureas, polyamides, acrylic resins, thermoplastics, polyphenylene oxide resins, thermoplastic polyesters, thermoplastic rubbers, partially-neutralized polymers, highly-neutralized polymers, and fully-neutralized polymers.

2. The golf ball of claim 1, wherein the core comprises a solid, liquid, or gel-filled center and an outer core layer.
3. The golf ball of claim 1, further comprising an intermediate layer comprising an ionomeric material, vinyl resins, polyolefins, polyurethanes, polyureas, polyamides, acrylic resins, thermoplastics, polyphenylene oxide resins, thermoplastic polyesters, thermoplastic rubbers, partially-neutralized polymers, highly-neutralized polymers, or fully-neutralized polymers.
4. The golf ball of claim 1, wherein the magnesium salt of pentachlorothiophenol is present in an amount from about 0.1 pph to about 0.75 pph.
5. The golf ball of claim 1, wherein the golf ball has a coefficient of restitution of greater than about 0.800.
6. The golf ball of claim 1, wherein the golf ball further comprises a water vapor barrier layer having a water vapor transmission rate of about 0.45 grams·mm/m<sup>2</sup>·day or less.
7. The golf ball of claim 1, wherein the polybutadiene composition further comprises between about 15 pph and about 35 pph of a salt of an  $\alpha,\beta$ -unsaturated carboxylic acid, between about 0.1 pph and about 1.2 pph of an organic peroxide, and a filler.
8. The golf ball of claim 1, wherein the polyurethane or polyurea comprises a prepolymer formed of a polyisocyanate and a polyol, and a curing agent.
9. The golf ball of claim 8, wherein the prepolymer and curing agent are saturated.
10. The golf ball of claim 1, wherein the polyurethane or polyurea comprises at least one of a UV absorber, a hindered amine light stabilizer, or an optical brightener.
11. A golf ball comprising:  
a core having a diameter of about 1.50 inches or greater and a compression of between about 40 and about 80, the core consisting of:  
a center; and  
an outer core layer,  
wherein at least one of the core or the outer core layer comprises a polybutadiene rubber composition comprising a magnesium salt of pentachlorothiophenol; an outer cover having a thickness of less than about 0.04 inches and comprising a castable polyurethane or polyurea composition; and  
an inner cover layer disposed between the core and the outer cover layer, the inner cover layer having a thickness of about 0.04 inches or less and comprising an ionomeric material, vinyl resins, polyolefins, polyurethanes, polyureas, polyamides, acrylic resins, thermoplastics, polyphenylene oxide resins, thermoplastic polyesters, thermoplastic rubbers, partially-neutralized polymers, highly-neutralized polymers, or fully-neutralized polymers.
12. The golf ball of claim 11, wherein the core has an outer diameter of between about 1.54 inches and about 1.61 inches.
13. The golf ball of claim 12, wherein the outer core layer further comprises ionomers, vinyl resins, polyolefins, polyurethanes, polyureas, polyamides, acrylic resins, thermoplastics, polyphenylene oxide resins, thermoplastic polyesters, thermoplastic rubbers, crosslinked polybutadiene rubber, partially-neutralized polymers, highly-neutralized polymers, or fully-neutralized polymers.
14. The golf ball of claim 11, wherein the golf ball has a coefficient of restitution of greater than about 0.800.
15. The golf ball of claim 11, wherein the core has a compression of between about 55 and about 70, and the golf ball has a coefficient of restitution of greater than about 0.800.

## 25

16. The golf ball of claim 11, wherein the polybutadiene composition further comprises between about 15 pph and about 35 pph of a salt of an  $\alpha,\beta$ -unsaturated carboxylic acid, between about 0.1 pph and about 0.75 pph of an organic peroxide, and a filler.

17. The golf ball of claim 11, wherein the polyurethane or polyurea composition comprises a prepolymer formed of a polyisocyanate and a polyol, and a curing agent.

18. The golf ball of claim 17, wherein at least one of the prepolymer and curing agent are saturated.

19. The golf ball of claim 17, wherein the polyurethane or polyurea composition comprises at least one of a UV absorber, a hindered amine light stabilizer, or an optical brightener.

20. A golf consisting of:

a core having a diameter of about 1.50 inches or greater, a compression of about 80 or less, and comprises a polybutadiene rubber composition comprising a magnesium salt of a halogenated thiophenol; and at least one cover layer comprising ionomers, vinyl resins, polyolefins, polyurethanes, polyureas, polyamides, acrylic resins, thermoplastics, polyphenylene oxide resins, thermoplastic polyesters, thermoplastic rubbers, partially-neutralized polymers, highly-neutralized polymers, fully-neutralized polymers, polyurethanes, or polyureas, and having a thickness of about 0.05 inches or less.

## 26

21. The golf ball of claim 20, wherein the halogenated thiophenol is selected from the group consisting of pentafluorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol 2,3,4-fluorothiophenol; 3,4,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; 15 pentabromothiophenol; 2-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,4,5-tetraiodothiophenol; and 2,3,5,6-tetraiodothiophenol.

\* \* \* \* \*